

No. 695,423.

Patented Mar. 11, 1902.

F. J. WARREN.  
STREET PAVEMENT.

(Application filed Jan. 10, 1902.)

(No Model.)



Fig. 1.



Fig. 2.

WITNESSES:

J. M. Dolan  
Saul Sippurstein

INVENTOR=  
Frederick J. Warren  
by his attorney  
Clarke & Raymond

# UNITED STATES PATENT OFFICE.

FREDERICK J. WARREN, OF NEWTON, MASSACHUSETTS.

## STREET-PAVEMENT.

SPECIFICATION forming part of Letters Patent No. 695,423, dated March 11, 1902.

Application filed January 10, 1902. Serial No. 89,164. (No specimens.)

*To all whom it may concern:*

Be it known that I, FREDERICK J. WARREN, a citizen of the United States, and a resident of Newton, in the county of Middlesex and 5 State of Massachusetts, have invented a new and useful Improvement in Street-Pavements, of which the following is a full, clear, and exact description, reference being had to the accompanying drawings, forming a part of 10 this specification, in explaining its nature.

The invention relates to any type of street pavement or roadway which is adapted to be surface-finished in the manner hereinafter indicated.

15 The object of the invention is to provide such pavements with a wearing-surface which shall possess first of all the property of great resistance to wear and which shall also act to preserve the portion of the pavement below which acts as a foundation and support 20 for it. Ordinarily the said foundation or support, or the portion of it to which the wearing-surface is applied, would be of a bituminous nature and would furnish the principal part of the body of the pavement, or at 25 any rate the upper part thereof, and my invention has nothing to do with this portion of the pavement, excepting that in order to use my invention most successfully it is necessary that this part of the pavement should 30 be suitably constructed. To the surface of a pavement so prepared I apply a wearing-surface consisting of a bituminous cement relatively pure and combined with iron or 35 steel filings, chips, or particles intimately associated with one or more layers of coatings of the bituminous cement. The cement must be in a fluid condition and may be either hot or cold when applied. It serves to combine 40 together the iron or steel fragments and to also seal the more or less cellular structure of the foundation against atmospheric influences. The nature of the metal particles is such that when combined with the cement 45 there is formed a tough, hard, durable water and weather proof surfacing which readily unites with the foundation upon which it is placed and which possesses enormous power of resisting wear of traffic, in conjunction with 50 great preservative power in protecting the main body of the pavement from the ordinary

destructive influences aside from traffic wear to which it is subjected.

I will now describe the invention in connection with the drawings forming a part of 55 this specification, in which—

Figure 1 is a view in cross vertical section of a street-pavement having the features of my invention. Fig. 2 is a view in vertical section of a portion thereof enlarged. 60

In the drawings a conventional pavement is represented, the section A of which is of a bituminous composition, consisting of asphalt, coal-tar, or any other similar vehicle combined with an earthy, concrete, or stony base and 65 in the usual proportions. This section of the pavement is prepared and laid in the ordinary manner and ordinarily would supply the ordinary or wearing section of the pavement. A pavement of this composition is more or 70 less cellular or filled with pores and to that extent is defective in that it invites attacks from atmospheric influences. To this section of the pavement is applied the wearing-surface B. This consists of any desired number of coats of fluid bitumen, either hot or 75 cold, as may be desired, and affixed to the surface of the said section B in any desired manner, but so as to be intimately connected and combined therewith and to evenly and uniformly cover it. With one or more of these 80 coatings of bitumen I combine iron or steel filings, particles, or fragments in any desired proportion and so as to make a composition which shall have a large proportion of its 85 body of metal. This is applied to the surface in the same manner that the other coatings are applied and may be used without them, if desired, and may be covered by one or more of them, if required. The effect is to 90 produce a pavement having a wearing-surface which has the power to resist traffic wear which iron or steel may have and so applied to the supporting-foundation as not to expose large pieces or sections of the metal 95 in an objectionable way, but which so combine as to make a continuous metal and bituminous layer throughout the surfacing of the pavement. This not only serves to receive the wear of traffic, but is practically imper- 100 vious to atmospheric influences, as well as not to be disintegrated or rotted by the weather.

It likewise serves to protect the foundation below it from the action of the weather and from wear, so that the integrity of the foundation is maintained and the durability of the entire pavement is very much increased.

I have spoken of the use of iron and steel filings, particles, and pieces, and I would say that the same waste of any other metal may be used for this purpose and that they may be combined with the iron and the steel filings, particles, and pieces, or not, as may be desired, and that the iron may be used apart from the steel, and vice versa, when preferred.

In lieu of mixing the iron and steel chips and particles with a bituminous cement in advance of the application of the metallized compound to the surface of the pavement or foundation I would say that they may be applied separately to the said pavement or foundation surface and combined together thereon, in which event there would be applied the bituminous cement in one or more coatings, and the metal chips or pieces would be spread thereon to any desired thickness or extent and then combined therewith by sweeping, pressure, or other mechanical means and by other coats or coatings of the bituminous cement, and this method of constructing the surface may be continued to any desired extent by the application of subsequent layers or coatings to the bituminous cement and of the metal chips or pieces until any desired thickness of wearing surface or body is secured.

In some instances grains of stone, cracked or otherwise, may be combined with the metal chips or filings and to any extent desired, so that the wearing-surface would then consist of iron or steel chips and filings, or either, stony grains or elements, and a combining vehicle of bituminous cement.

Having thus fully described my invention, I claim and desire to secure by Letters Patent of the United States—

1. The application to the wearing-surface of a bituminous street-pavement having a cellular or porous character for the purpose of closing its pores, preserving its life and increasing its resistance to wear, of a cell and pore sealing coating of bituminous cement and iron, steel or other metal filings, chips or particles.

2. The application to the wearing-surface of a bituminous street-pavement of a thin coating of bituminous cement applied thereto in a plastic condition and combined while plastic with metal filings, chips or particles and whereby the wearing-surface is provided with increased durability.

3. The application to the wearing-surface of a bituminous street-pavement of a layer or coating of relatively pure bitumen, a layer or coating of iron, steel or other metal filings, chips or particles and a bituminous cement intimately commingled and a layer or coating of relatively pure bitumen applied to the surface of the metal and bituminous layer.

4. The application to the wearing-surface of a bituminous street-pavement of a coating consisting of a composition of bitumen, stony ingredients and iron or steel filings, chips or particles mingled to form a homogeneous body of stone, metal and bitumen, and whereby the wearing-surface of the pavement is provided with increased durability and also with frictional properties.

FREDERICK J. WARREN.

Witnesses:

F. F. RAYMOND, 2d,  
J. M. DOLAN.